# EUROPEAN PATENT APPLICATION

(11) **EP 3 264 183 A1**
(43) Date of publication of application: **03.01.2018**
(21) Application number: 17177542.2
(22) Date of filing: 22.06.2017
(51) Int. Cl.: G03G 5/147

(54) **FLUORINATED STRUCUTURED ORGANIC FILM LAYER PHOTORECEPTOR LAYERS**

(30) Priority: 30.06.2016 US 201615198680
(71) Applicant: Xerox Corporation, Rochester, NY 14644 (US)
(72) Inventor: MCGUIRE, Gregory M., Mississauga, Ontario L5K 2L1 (CA); YANG, Suxia, Mississauga, Ontario L5J 1T2 (CA); HU, Nan-Xing, Oakville, Ontario L6H 7V3 (CA); SAVAGE, Edward C., Webster, NY New York 14580 (US); HEDRICK, Robert W., Spencerport, NY New York 14559 (US)
(74) Representative: Gill Jennings & Every LLP

(57) **Abstract**

Disclosed herein is an imaging member that includes a substrate, a charge generating layer, a charge transport layer; and an outermost layer comprising a structured organic film (SOF) comprising a fluorinated molecular building block and a hole molecular building block, wherein the fluorinated molecular building block is present in the SOF of the outermost layer in an amount of from about 1 weight percent to about 20 weight percent of the SOF.

## Description

### BACKGROUND

### Field of Use

The present disclosure relates to protective overcoats for imaging members. More particularly, there is provided a structured organic film used an overcoat for a photoreceptor.

### Background

In electrophotography, electrophotographic imaging or electrostatographic imaging, the surface of an electrophotographic plate, drum, belt or the like (imaging member or photoreceptor) containing a photoconductive insulating layer on a conductive layer is first uniformly electrostatically charged. The imaging member is exposed to a pattern of activating electromagnetic radiation, such as light. The radiation selectively dissipates the charge on the illuminated areas of the photoconductive insulating layer while leaving behind an electrostatic latent image on the non-illuminated areas. This electrostatic latent image may then be developed to form a visible image by depositing finely divided electroscopic marking particles on the surface of the photoconductive insulating layer. The resulting visible image may then be transferred from the imaging member directly or indirectly (such as by a transfer or other member) to a print substrate, such as transparency or paper. The imaging process may be repeated many times with reusable imaging members.

Although excellent toner images may be obtained with multilayered belt or drum photoreceptors, it has been found that as more advanced, higher speed electrophotographic copiers, duplicators, and printers are developed, there is a greater demand on print quality. The delicate balance in charging image and bias potentials, and characteristics of the toner and/or developer, must be maintained. This places additional constraints on the quality of photoreceptor manufacturing, and thus on the manufacturing yield.

Imaging members are generally exposed to repetitive electrophotographic cycling, which subjects the exposed charged transport layer or alternative top layer thereof to mechanical abrasion, chemical attack and heat. This repetitive cycling leads to gradual deterioration in the mechanical and electrical characteristics of the exposed charge transport layer. Physical and mechanical damage during prolonged use, especially the formation of surface scratch defects, is among the chief reasons for the failure of belt photoreceptors. Therefore, it is desirable to improve the mechanical robustness of photoreceptors, and particularly, to increase their scratch resistance, thereby prolonging their service life. Additionally, it is desirable to increase resistance to light shock so that image ghosting, background shading, and the like is minimized in prints.

Providing a protective overcoat layer is a conventional means of extending the useful life of photoreceptors. Conventionally, for example, a polymeric anti-scratch and crack overcoat layer has been utilized as a robust overcoat design for extending the lifespan of photoreceptors. However, the conventional overcoat layer formulation exhibits ghosting and background shading in prints. Improving light shock resistance will provide a more stable imaging member resulting in improved print quality.

Despite the various approaches that have been taken for forming imaging members, there remains a need for improved imaging member design, to provide improved imaging performance and longer lifetime, reduce human and environmental health risks, and the like.

### SUMMARY

According to an embodiment, there is provided an imaging member that includes a substrate, a charge generating layer, a charge transport layer; and an outermost layer comprising a structured organic film (SOF) comprising a fluorinated molecular building block and a hole molecular building block, wherein the fluorinated molecular building block is present in the SOF of the outermost layer in an amount of from about 1 weight percent to about 20 weight percent of the SOF.

According to another embodiment, there is provided an electrostatographic apparatus that includes an imaging member having an outermost layer. The outermost layer is a structured organic film (SOF) including a plurality of fluorinated molecular building blocks and a plurality of hole molecular building blocks, wherein the fluorinated molecular building blocks are present in the SOF in an amount of from about 1 weight percent to about 20 weight percent of the SOF. The electrostatogrpahic device includes a charging unit to impart an electrostatic charge on the imaging member, an exposure unit to create an electrostatic latent image on the imaging member, an image material delivery unit to create an image on the imaging member and a transfer unit to transfer the image from the imaging member. The electrostographic device can optionally include a cleaning unit.

According to another embodiment, there is provided an imaging member including a substrate, a charge generating layer, a charge transport layer and an outermost layer. The outermost layer is a structured organic film (SOF) including fluorinated molecular building blocks and hole molecular building blocks, wherein the fluorinated molecular building blocks are present in the SOF in an amount of from about 1 weight percent to about 10 weight percent of the SOF.

### BRIEF DESCRIPTION OF THE DRAWINGS

The accompanying drawings, which are incorporated in and constitute a part of this specification, illustrate several embodiments of the present teachings and together with the description, serve to explain the principles of the present teachings.
FIG.1 represents a simplified side view of an exemplary photoreceptor that incorporates a FSOF of the present disclosure.
FIG. 2 represents a simplified side view of a second exemplary photoreceptor that incorporates a FSOF of the present disclosure.
FIG. 3 represents a simplified side view of a third exemplary photoreceptor that incorporates a FSOF of the present disclosure.

It should be noted that some details of the FIGS. have been simplified and are drawn to facilitate understanding of the embodiments rather than to maintain strict structural accuracy, detail, and scale.

### DESCRIPTION OF THE EMBODIMENTS

Reference will now be made in detail to embodiments of the present teachings, examples of which are illustrated in the accompanying drawings. Wherever possible, the same reference numbers will be used throughout the drawings to refer to the same or like parts.

In the following description, reference is made to the accompanying drawings that form a part thereof, and in which is shown by way of illustration specific exemplary embodiments in which the present teachings may be practiced. These embodiments are described in sufficient detail to enable those skilled in the art to practice the present teachings and it is to be understood that other embodiments may be utilized and that changes may be made without departing from the scope of the present teachings. The following description is, therefore, merely illustrative.

Illustrations with respect to one or more implementations, alterations and/or modifications can be made to the illustrated examples without departing from the spirit and scope of the appended claims. In addition, while a particular feature may have been disclosed with respect to only one of several implementations, such feature may be combined with one or more other features of the other implementations as may be desired and advantageous for any given or particular function. Furthermore, to the extent that the terms "including", "includes", "having", "has", "with", or variants thereof are used in either the detailed description and the claims, such terms are intended to be inclusive in a manner similar to the term "comprising." The term "at least one of" is used to mean one or more of the listed items can be selected.

Notwithstanding that the numerical ranges and parameters setting forth the broad scope of embodiments are approximations, the numerical values set forth in the specific examples are reported as precisely as possible. Any numerical value, however, inherently contains certain errors necessarily resulting from the standard deviation found in their respective testing measurements. Moreover, all ranges disclosed herein are to be understood to encompass any and all sub-ranges subsumed therein. For example, a range of "less than 10" can include any and all sub-ranges between (and including) the minimum value of zero and the maximum value of 10, that is, any and all sub-ranges having a minimum value of equal to or greater than zero and a maximum value of equal to or less than 10, e.g., 1 to 5. In certain cases, the numerical values as stated for the parameter can take on negative values. In this case, the example value of range stated as "less than 10" can assume negative values, e.g. - 1, -2, -3, -10, -20, -30, etc.

The term "fluorinated SOF" refers, for example, to a SOF that contains fluorine atoms covalently bonded to one or more segment types or linker types of the SOF. The fluorinated SOFs of the present disclosure may further comprise fluorinated molecules that are not covalently bound to the framework of the SOF, but are randomly distributed in the fluorinated SOF composition (i.e., a composite fluorinated SOF). However, an SOF, which does not contain fluorine atoms covalently bonded to one or more segment types or linker types of the SOF, that merely includes fluorinated molecules that are not covalently bonded to one or more segments or linkers of the SOF is a composite SOF, not a fluorinated SOF.

U.S. Patent 8,372,566, incorporated herein by reference, discloses FSOF films containing fluorinated segments and electroactive segments. The fluorinated segments are at least 25 weight percent of the film. It has been found that lowering the fluorine content in the film improves wear and increases life of the photoreceptor and improves overall image quality.

Disclosed herein is a Fluorinated Structured Organic Film (FSOF) wherein the fluorine molecular building block component is from about 1 weight percent to about 20 weight percent of the FSOF. The films exhibit extraordinarily low wear rates while still maintaining low surface energy characteristics and excellent print quality. The low wear rate enables well over 1 million prints before wearing through the overcoat layer. Furthermore, the extremely hard surface shows extreme resistance to scratching and remains undamaged which enables life of machine use as well as the option for re-man usage.

In embodiments, the fluorine molecular building block component of the FSOF of the present disclosure may be of from about 1 % to about 20 % by weight, such as about 1 % to about 10 % by weight, or about 1 % to about 5 % by weight of the FSOF.

In embodiments, the fluorine content of the FSOF of the present disclosure may be of from about 1 % to about 15 % by weight of the FSOF, such as about 1 % to about 10 % by weight, or about 1 % to about 5 % by weight of the FSOF.

In embodiments, the FSOF may be made by the reaction of one or more suitable molecular building blocks, where at least one of the molecular building block segments comprises fluorine atoms.

In embodiments, the imaging members and/or photoreceptors of the present disclosure comprise an outermost layer that comprises a FSOF in which a first segment having hole transport properties (hole molecular building block), which may be obtained from the reaction of a fluorinated molecular building block.

In embodiments, the outermost layer of the imaging members and/or photoreceptors comprises an FSOF wherein the microscopic arrangement of segments is patterned. The term "patterning" refers, for example, to the sequence in which segments are linked together. A patterned fluorinated SOF would therefore embody a composition wherein, for example, segment A (having hole transport molecule functions) is only connected to segment B (which is a fluorinated molecular building block), and conversely, segment B is only connected to segment A.

In principle a patterned FSOF may be achieved using any number of segment types. The patterning of segments may be controlled by using molecular building blocks whose functional group reactivity is intended to compliment a partner molecular building block and wherein the likelihood of a molecular building block to react with itself is minimized. The aforementioned strategy to segment patterning is non-limiting.

In embodiments, the outermost layer of the imaging members and/or photoreceptors comprises patterned FSOFs having different degrees of patterning. For example, the patterned FSOF may exhibit full patterning, which may be detected by the complete absence of spectroscopic signals from building block functional groups. In other embodiments, the patterned FSOFs having lowered degrees of patterning wherein domains of patterning exist within the FSOF.

In embodiments, the fluorine content of the FSOFs comprised in the outermost layer of the imaging members and/or photoreceptors of the present disclosure may be distributed throughout the FSOF in a heterogeneous manner, including various patterns, wherein the concentration or density of the fluorine content is reduced in specific areas, such as to form a pattern of alternating bands of high and low concentrations of fluorine of a given width. Such pattering maybe accomplished by utilizing a mixture of molecular building blocks sharing the same general parent molecular building block structure but differing in the degree of fluorination (i.e., the number of hydrogen atoms replaced with fluorine) of the building block.

A description of various exemplary molecular building blocks, linkers, SOF types, capping groups, strategies to synthesize a specific SOF type with exemplary chemical structures, building blocks whose symmetrical elements are outlined, and classes of exemplary molecular entities and examples of members of each class that may serve as molecular building blocks for SOFs are detailed in U.S. patent application Ser. Nos. 12/716,524; 12/716,449; 12/716,706; 12/716,324; 12/716,686; 12/716,571; 12/815,688; 12/845,053; 12/845,235; 12/854,962; 12/854,957; and 12/845,052 entitled "Structured Organic Films," "Structured Organic Films Having an Added Functionality," "Mixed Solvent Process for Preparing Structured Organic Films," "Composite Structured Organic Films," "Process For Preparing Structured Organic Films (SOFs) Via a Pre-SOF," "Electronic Devices Comprising Structured Organic Films," "Periodic Structured Organic Films," "Capped Structured Organic Film Compositions," "Imaging Members Comprising Capped Structured. Organic Film Compositions," "Imaging Members for Ink-Based Digital Printing Comprising Structured Organic Films," "Imaging Devices Comprising Structured Organic Films," and "Imaging Members Comprising Structured Organic Films," respectively; and U.S. Provisional Application No. 61/157,411, entitled "Structured Organic Films" filed Mar. 4, 2009, the disclosures of which are totally incorporated herein by reference in their entireties.

In embodiments, fluorinated molecular building blocks may be obtained from the fluorination of any of the above "parent" non-fluorinated molecular building blocks (e.g., molecular building blocks detailed in U.S. patent application Ser. Nos. 12/716,524; 12/716,449; 12/716,706; 12/716,324; 12/716,686; 12/716,571; 12/815,688; 12/845,053; 12/845,235; 12/854,962; 12/854,957; and 12/845,052, previously incorporated by reference) by known processes. For example, "parent" non-fluorinated molecular building blocks may be fluorinated via elemental fluorine at elevated temperatures, such as greater than about 150.degree. C., or by other known process steps to form a mixture of fluorinated molecular building blocks having varying degrees of fluorination, which may be optionally purified to obtain an individual fluorinated molecular building block. Alternatively, fluorinated molecular building blocks may be synthesized and/or obtained by simple purchase of the desired fluorinated molecular building block. The conversion of a "parent" non-fluorinated molecular building block into a fluorinated molecular building block may take place under reaction conditions that utilize a single set or range of known reaction conditions, and may be a known one step reaction or known multi-step reaction. Exemplary reactions may include one or more known reaction mechanisms, such as an addition and/or an exchange.

### Molecular Building Block

The FSOFs of the present disclosure comprise molecular building blocks having a segment (S) and functional groups (Fg). Molecular building blocks require at least two functional groups (x≥2) and may comprise a single type or two or more types of functional groups. Functional groups are the reactive chemical moieties of molecular building blocks that participate in a chemical reaction to link together segments during the FSOF forming process. A segment is the portion of the molecular building block that supports functional groups and comprises all atoms that are not associated with functional groups. Further, the composition of a molecular building block segment remains unchanged after SOF formation.

Molecular building block symmetry relates to the positioning of functional groups (Fgs) around the periphery of the molecular building block segments. Without being bound by chemical or mathematical theory, a symmetric molecular building block is one where positioning of Fgs may be associated with the ends of a rod, vertexes of a regular geometric shape, or the vertexes of a distorted rod or distorted geometric shape. For example, the most symmetric option for molecular building blocks containing four Fgs are those whose Fgs overlay with the corners of a square or the apexes of a tetrahedron.

Use of symmetrical building blocks is practiced in embodiments of the present disclosure for two reasons: (1) the patterning of molecular building blocks may be better anticipated because the linking of regular shapes is a better understood process in reticular chemistry, and (2) the complete reaction between molecular building blocks is facilitated because for less symmetric building blocks errant conformations/orientations may be adopted which can possibly initiate numerous linking defects within FSOFs.

The FSOFs in the outermost layer of the imaging members and/or photoreceptors of the present disclosure may be made from versions of any of the molecular building blocks, segments, and/or linkers wherein one or more hydrogen(s) in the molecular building blocks are replaced with fluorine.

Non-limiting examples of various classes of exemplary molecular entities, that may serve as molecular building blocks for SOFs of the present disclosure include building blocks containing a carbon or silicon atomic core; building blocks containing alkoxy cores; building blocks containing a nitrogen or phosphorous atomic core; building blocks containing aryl cores; building blocks containing carbonate cores; building blocks containing carbocyclic-, carbobicyclic-, or carbotricyclic core; and building blocks containing an oligothiophene core.

In embodiments, exemplary fluorinated molecular building blocks may be obtained from the fluorination building blocks containing a carbon or silicon atomic core; building blocks containing alkoxy cores; building blocks containing a nitrogen or phosphorous atomic core; building blocks containing aryl cores; building blocks containing carbonate cores; building blocks containing carbocyclic-, carbobicyclic-, or carbotricyclic core; and building blocks containing an oligothiophene core. Such fluorinated molecular building blocks may be obtained from the fluorination of a non-fluorinated molecular building block with elemental fluorine at elevated temperatures, such as greater than about 150°C., or by other known process steps, or by simple purchase of the desired fluorinated molecular building block.

### Functional Group

Functional groups are the reactive chemical moieties of molecular building blocks that participate in a chemical reaction to link together segments during the FSOF forming process. Functional groups may be composed of a single atom, or functional groups may be composed of more than one atom. The atomic compositions of functional groups are those compositions normally associated with reactive moieties in chemical compounds. Non-limiting examples of functional groups include halogens, alcohols, ethers, ketones, carboxylic acids, esters, carbonates, amines, amides, imines, ureas, aldehydes, isocyanates, tosylates, alkenes, alkynes and the like.

Molecular building blocks contain a plurality of chemical moieties, but only a subset of these chemical moieties are intended to be functional groups during the FSOF forming process. Whether or not a chemical moiety is considered a functional group depends on the reaction conditions selected for the SOF forming process. Functional groups (Fg) denote a chemical moiety that is a reactive moiety, that is, a functional group during the SOF forming process.

In the FSOF forming process, the composition of a functional group will be altered through the loss of atoms, the gain of atoms, or both the loss and the gain of atoms; or, the functional group may be lost altogether. In the FSOF, atoms previously associated with functional groups become associated with linker groups, which are the chemical moieties that join together segments. Functional groups have characteristic chemistries and those of ordinary skill in the art can generally recognize in the present molecular building blocks the atom(s) that constitute functional group(s). It should be noted that an atom or grouping of atoms that are identified as part of the molecular building block functional group may be preserved in the linker group of the FSOF. Linker groups are described below.

Capping units of the present disclosure are molecules that 'interrupt' the regular network of covalently bonded building blocks normally present in an FSOF. Capped FSOF compositions are tunable materials whose properties can be varied through the type and amount of capping unit introduced. Capping units may comprise a single type or two or more types of functional groups and/or chemical moieties.

In embodiments, the FSOF comprises a plurality of segments, where all segments have an identical structure, and a plurality of linkers, which may or may not have an identical structure, wherein the segments that are not at the edges of the FSOF are connected by linkers to at least three other segments and/or capping groups. In embodiments, the FSOF comprises a plurality of segments where the plurality of segments comprises at least a first and a second segment that are different in structure, and the first segment is connected by linkers to at least three other segments and/or capping groups when it is not at the edge of the FSOF.

In embodiments, the FSOF comprises a plurality of linkers including at least a first and a second linker that are different in structure, and the plurality of segments either comprises at least a first and a second segment that are different in structure, where the first segment, when not at the edge of the FSOF, is connected to at least three other segments and/or capping groups, wherein at least one of the connections is via the first linker, and at least one of the connections is via the second linker; or comprises segments that all have an identical structure, and the segments that are not at the edges of the FSOF are connected by linkers to at least three other segments and/or capping groups, wherein at least one of the connections is via the first linker, and at least one of the connections is via the second linker.

A segment is the portion of the molecular building block that supports functional groups and comprises all atoms that are not associated with functional groups. Further, the composition of a molecular building block segment remains unchanged after FSOF formation. In embodiments, the FSOF may contain a first segment having a structure the same as or different from a second segment. In other embodiments, the structures of the first and/or second segments may be the same as or different from a third segment, forth segment, fifth segment, etc. A segment is also the portion of the molecular building block that can provide an inclined property. Inclined properties are described later in the embodiments.

A linker is a chemical moiety that emerges in a FSOF upon chemical reaction between functional groups present on the molecular building blocks and/or capping unit.

A linker may comprise a covalent bond, a single atom, or a group of covalently bonded atoms. The former is defined as a covalent bond linker and may be, for example, a single covalent bond or a double covalent bond and emerges when functional groups on all partnered building blocks are lost entirely. The latter linker type is defined as a chemical moiety linker and may comprise one or more atoms bonded together by single covalent bonds, double covalent bonds, or combinations of the two. Atoms contained in linking groups originate from atoms present in functional groups on molecular building blocks prior to the SOF forming process. Chemical moiety linkers may be well-known chemical groups such as, for example, esters, ketones, amides, imines, ethers, urethanes, carbonates, and the like, or derivatives thereof.

For example, when two hydroxyl (--OH) functional groups are used to connect segments in a FSOF via an oxygen atom, the linker would be the oxygen atom, which may also be described as an ether linker. In embodiments, the SOF may contain a first linker having a structure the same as or different from a second linker. In other embodiments, the structures of the first and/or second linkers may be the same as or different from a third linker, etc.

Use of symmetrical building blocks is practiced in embodiments of the present disclosure for two reasons: (1) the patterning of molecular building blocks is better anticipated because the linking of regular shapes is a better understood process in reticular chemistry, and (2) the complete reaction between molecular building blocks is facilitated because for less symmetric building blocks errant conformations/orientations may be adopted which can possibly initiate numerous linking defects within FSOFs.

In embodiments, the outermost layer of the imaging members and/or photoreceptors comprises patterned FSOFs having different degrees of patterning. For example, the patterned FSOF may exhibit full patterning, which may be detected by the complete absence of spectroscopic signals from building block functional groups. In other embodiments, the patterned FSOFs having lowered degrees of patterning wherein domains of patterning exist within the FSOF.

The fluorinated molecular building blocks may include, for example, α, ω-fluoroalkyldiols of the general structure: where n is an integer having a value of 1 or more, such as from 1 to about 100, or 1 to about 60, or about 2 to about 30, or about 4 to about 10; or fluorinated alcohols of the general structure HOCH₂(CF₂)ₙCH₂OH and their corresponding dicarboxylic acids and aldehydes, where n is an integer having a value of 1 or more, such as from 1 to about 100, or 1 to about 60, or about 2 to about 30, or about 4 to about 10; tetrafluorohydroquinone; perfluoroadipic acid hydrate, 4,4'-(hexafluoroisopropylidene)diphthalic anhydride; 4,4'-(hexafluoroisopropylidene)diphenol, and the like.

Examples of the fluorinated building blocks include fluorinated diols selected from the group consisting of: 1,1,8,8-dodecafluoro-1,8-octanediol, 2,2,3,3,4,4,5,5-octafluoro-1,6-hexanediol, 2,2,3,3,4,4,5,5,6,6,7,7-dodecanfluoro-1,8-octanediol, 2,2,3,3,4,4,5,5,6,6,7,7,8,8,9,9-perfluorodecane-1,10-diol, (2,3,5,6-tetrafluoro-4-hydroxymethyl-phenyl)-methanol, 2,2,3,3-tetrafluoro-1,4-butanediol, 2,2,3,3,4,4-hexafluoro-1,5-pentanedial, and 2,2,3,3,4,4,5,5,6,6,7,7,8,8-tetradecafluoro-1,9-nonanediol.

The term electroactive refers, for example, to the property to transport electrical charge (electrons and/or holes). Examples of hole transport building blocks having electroactive properties, include N,N,N',N'-tetrakis-[(4-hydroxymethyl)phenyl]-biphenyl-4,4'-diamin- e, having a hydroxyl functional group (--OH) and upon reaction results in a segment of N,N,N',N'-tetra-(p-tolyl)biphenyl-4,4'-diamine; and/or N,N'-diphenyl-N,N'-bis-(3-hydroxyphenyl)-biphenyl-4,4'-diamine, having a hydroxyl functional group (--OH) and upon reaction results in a segment of N,N,N',N'-tetraphenyl-biphenyl-4,4'-diamine.

Hole transport building blocks having added functionality may be obtained by selecting segment cores such as, for example, triarylamines, hydrazones (U.S. Pat. No. 7,202,002 B2 to Tokarski et al.), and enamines (U.S. Pat. No. 7,416,824 B2 to Kondoh et al.) with the following general structures:

The segment core comprising a triarylamine being represented by the following general formula: wherein Ar¹, Ar², Ar³, Ar⁴ and Ar⁵ each independently represents a substituted or unsubstituted aryl group, or Ar⁵ independently represents a substituted or unsubstituted arylene group, and k represents 0 or 1. Ar⁵ may be further defined as, for example, a substituted phenyl ring, substituted/unsubstituted phenylene, substituted/unsubstituted monovalently linked aromatic rings such as biphenyl, terphenyl, and the like, or substituted/unsubstituted fused aromatic rings such as naphthyl, anthranyl, phenanthryl, and the like.

Segment cores comprising arylamines with hole transport added functionality include, for example, aryl amines such as triphenylamine, N,N,N',N'-tetraphenyl-(1,1'-biphenyl)-4,4'-diamine, N,N-diphenyl-N,N'-bis(3-methylphenyl)-(1,1'-biphenyl)-4,4'-diamine, N,N'-bis(4-butylphenyl)-N,N'-diphenyl-[p-terphenyl]-4,4"-diamine; hydrazones such as N-phenyl-N-methyl-3-(9-ethyl)carbazyl hydrazone and 4-diethyl amino benzaldehyde-1,2-diphenyl hydrazone; and oxadiazoles such as 2,5-bis(4-N,N'-diethylaminophenyl)-1,2,4-oxadiazole, stilbenes, and the like.

The segment core comprising a hydrazone being represented by the following general formula: wherein Ar¹, Ar², and Ar³ each independently represents an aryl group optionally containing one or more substituents, and R represents a hydrogen atom, an aryl group, or an alkyl group optionally containing a substituent; wherein at least two of Ar¹, Ar², and Ar³ comprises a Fg (previously defined); and a related oxadiazole being represented by the following general formula: wherein Ar and Ar¹ each independently represent an aryl group that comprises a Fg (previously defined).

The segment core comprising an enamine being represented by the following general formula: wherein Ar¹, Ar², Ar³, and Ar⁴ each independently represents an aryl group that optionally contains one or more substituents or a heterocyclic group that optionally contains one or more substituents, and R represents a hydrogen atom, an aryl group, or an alkyl group optionally containing a substituent; wherein at least two of Ar¹, Ar², Ar³, and Ar⁴ comprises a Fg (previously defined).

Examples of the hole molecular building block include N4,N4,N4',N4'-tetrakis(4-(methoxymethyl)phenyl)biphenyl-4,4'-diamine N,N,N',N'-tetra-(p-tolyl)biphenyl-4,4'-diamine: and N4,N4'-bis(3,4-dimethylphenyl)-N4,N4'-di-p-tolyl-[1,1'-biphenyl]-4,4'-diamine.

FSOFs having a rough, textured, or porous surface on the sub-micron to micron scale may also be hydrophobic. The rough, textured, or porous FSOF surface can result from dangling functional groups present on the film surface or from the structure of the FSOF. The type of pattern and degree of patterning depends on the geometry of the molecular building blocks and the linking chemistry efficiency. The feature size that leads to surface roughness or texture is from about 100 nm to about 10 µm, such as from about 500 nm to about 5 µm.

The process described herein utilizes solvents, and/or solvent mixtures. Solvents are used to dissolve or suspend the molecular building blocks and catalyst/modifiers in the reaction mixture. Solvent selection is generally based on balancing the solubility/dispersion of the molecular building blocks and a particular building block loading, the viscosity of the reaction mixture, and the boiling point of the liquid, which impacts the promotion of the wet layer to the dry SOF.

Solvents can include molecule classes such as alkanes (hexane, heptane, octane, nonane, decane, cyclohexane, cycloheptane, cyclooctane, decalin); mixed alkanes (hexanes, heptanes); branched alkanes (isooctane); aromatic compounds (toluene, o-, m-, p-xylene, mesitylene, nitrobenzene, benzonitrile, butylbenzene, aniline); ethers (benzyl ethyl ether, butyl ether, isoamyl ether, propyl ether); cyclic ethers (tetrahydrofuran, dioxane), esters (ethyl acetate, butyl acetate, butyl butyrate, ethoxyethyl acetate, ethyl propionate, phenyl acetate, methyl benzoate); ketones (acetone, methyl ethyl ketone, methyl isobutylketone, diethyl ketone, chloroacetone, 2-heptanone), cyclic ketones (cyclopentanone, cyclohexanone), amines (1°, 2°, or 3° amines such as butylamine, diisopropylamine, triethylamine, diisoproylethylamine; pyridine); amides (dimethylformamide, N-methylpyrrolidinone, N,N-dimethylformamide); alcohols (methanol, ethanol, n-, i-propanol, n-, t-butanol, 1-methoxy-2-propanol, hexanol, cyclohexanol, 3-pentanol, benzyl alcohol); nitriles (acetonitrile, benzonitrile, butyronitrile), halogenated aromatics (chlorobenzene, dichlorobenzene, hexafluorobenzene), halogenated alkanes (dichloromethane, chloroform, dichloroethylene, tetrachloroethane); and water.

Catalyst are utilized in the reaction mixture to assist the promotion of the wet layer to the dry FSOF. Selection and use of the optional catalyst depends on the functional groups on the molecular building blocks. Catalysts may be homogeneous (dissolved) or heterogeneous (undissolved or partially dissolved) and include Bronsted acids (HCl (aq), acetic acid, p-toluenesulfonic acid, amine-protected p-toluenesulfonic acid such as pyrridium p-toluenesulfonate, trifluoroacetic acid); Lewis acids (boron trifluoroetherate, aluminum trichloride); Bronsted bases (metal hydroxides such as sodium hydroxide, lithium hydroxide, potassium hydroxide; 1°, 2°, or 3° amines such as butylamine, diisopropylamine, triethylamine, diisoproylethylamine); Lewis bases (N,N-dimethyl-4-aminopyridine); metals (Cu bronze); metal salts (FeCl3, AuCl3); and metal complexes (ligated palladium complexes, ligated ruthenium catalysts). Typical catalyst loading ranges from about 0.01% to about 25%, such as from about 0.1% to about 5% of the molecular building block loading in the reaction mixture. The catalyst may or may not be present in the final SOF composition.

Optionally additives or secondary components, such as dopants, antioxidants and leveling agents may be present in the reaction mixture and wet layer. Such additives or secondary components may also be integrated into a dry SOF. Additives or secondary components can be homogeneous or heterogeneous in the reaction mixture and wet layer or in a dry SOF. Typical leveling agents include hydroxyl-functionalized silicone modified polyacrylates available as SILCLEAN® 3700 (BYK, Wallingford, Conn.).

### Process for Preparing a Fluorinated Structured Organic Film (FSOF)

The process for making FSOFs of the present disclosure typically comprises a number of activities or steps (set forth below) that may be performed in any suitable sequence or where two or more activities are performed simultaneously or in close proximity in time:
The process for preparing a FSOF includes:
   (a) preparing a liquid-containing reaction mixture comprising a plurality of molecular building blocks, each comprising a segment (where at least one segment may comprise fluorine and at least one of the resulting segments is electroactive, such as an HTM) and a number of functional groups, and optionally a pre-FSOF;
   (b) depositing the reaction mixture as a wet film;
   (c) promoting a change of the wet film including the molecular building blocks to a dry film comprising the FSOF comprising a plurality of the segments and a plurality of linkers arranged as a covalent organic framework, wherein at a macroscopic level the covalent organic framework is a film;
   (d) optionally removing the FSOF from the substrate to obtain a free-standing FSOF;
   (e) optionally processing the free-standing FSOF into a roll;
   (f) optionally cutting and seaming the FSOF into a belt; and (g) optionally performing the above SOF formation process(es) upon an SOF (which was prepared by the above SOF formation process(es)) as a substrate for subsequent SOF formation process(es).

The process for making capped FSOFs and/or composite FSOFs typically comprises a similar number of activities or steps (set forth above) that are used to make a non-capped FSOF. The capping unit and/or secondary component may be added during either step a, b or c, depending the desired distribution of the capping unit in the resulting FSOF. For example, if it is desired that the capping unit and/or secondary component distribution is substantially uniform over the resulting FSOF, the capping unit may be added during step a. Alternatively, if, for example, a more heterogeneous distribution of the capping unit and/or secondary component is desired, adding the capping unit and/or secondary component (such as by spraying it on the film formed during step b or during the promotion step of step c) may occur during steps b and c.

Representative structures of an electrophotographic imaging member (e.g., a photoreceptor) are shown in FIGS. 1-3. These imaging members are provided with an anti-curl layer 1, a supporting substrate 2, an electrically conductive ground plane 3, a charge blocking layer 4, an adhesive layer 5, a charge generating layer 6, a charge transport layer 7, an overcoating layer 8, and a ground strip 9. In FIG. 3, imaging layer 10 (containing both charge generating material and charge transport material) takes the place of separate charge generating layer 6 and charge transport layer 7.

As seen in the figures, in fabricating a photoreceptor, a charge generating material (CGM) and a charge transport material (CTM) may be deposited onto the substrate surface either in a laminate type configuration where the CGM and CTM are in different layers (e.g., FIGS. 1 and 2) or in a single layer configuration where the CGM and CTM are in the same layer (e.g., FIG. 3). In embodiments, the photoreceptors may be prepared by applying over the electrically conductive layer the charge generation layer 6 and, optionally, a charge transport layer 7. In embodiments, the charge generation layer and, when present, the charge transport layer, may be applied in either order.

### Photoconductor Layer Examples

### Anti Curl Layer

With reference to FIGS. 1, 2 and 3, an optional anti-curl layer 1, which comprises film-forming organic or inorganic polymers that are electrically insulating or slightly semiconductive, may be provided. The anti-curl layer provides flatness and/or abrasion resistance. The anti-curl layer is typically used in photoconductor belts.

Anti-curl layer 1 may be formed at the back side of the substrate 2, opposite the imaging layers. The anti-curl layer 1 may include, in addition to the film-forming resin, an adhesion promoter polyester additive. Examples of film-forming resins useful as the anti-curl layer include, but are not limited to, polyacrylate, polystyrene, poly(4,4'-isopropylidene diphenylcarbonate), poly(4,4'-cyclohexylidene diphenylcarbonate), mixtures thereof and the like.

The thickness of the anti-curl layer 1 is typically from about 3 micrometers to about 35 micrometers, such as from about 10 micrometers to about 20 micrometers, or about 14 micrometers.

### The Supporting Substrate

As indicated above, the photoreceptors are prepared by first providing a substrate 2, i.e., a support. The substrate may be opaque or substantially transparent and may comprise any additional suitable material(s) having given required mechanical properties, such as those described in U.S. Pat. Nos. 4,457,994; 4,871,634; 5,702,854; 5,976,744; and 7,384,717 the disclosures of which are incorporated herein by reference in their entireties.

The substrate 2 may comprise a layer of electrically non-conductive material or a layer of electrically conductive material, such as an inorganic or organic composition. If a non-conductive material is employed, it may be necessary to provide an electrically conductive ground plane over such non-conductive material. If a conductive material is used as the substrate, a separate ground plane layer may not be necessary.

The substrate may be flexible or rigid and may have any of a number of different configurations, such as, for example, a sheet, a scroll, an endless flexible belt, a web, a cylinder, and the like. The photoreceptor may be coated on a rigid, opaque, conducting substrate, such as an aluminum drum.

### The Electrically Conductive Ground Plane

As stated above, in embodiments, the photoreceptors prepared comprise a substrate that is either electrically conductive or electrically non-conductive. When a non-conductive substrate is employed, an electrically conductive ground plane 3 must be employed, and the ground plane acts as the conductive layer. When a conductive substrate is employed, the substrate may act as the conductive layer, although a conductive ground plane may also be provided.

If an electrically conductive ground plane is used, it is positioned over the substrate. Suitable materials for the electrically conductive ground plane include, for example, aluminum, zirconium, niobium, tantalum, vanadium, hafnium, titanium, nickel, stainless steel, chromium, tungsten, molybdenum, copper, and the like, and mixtures and alloys thereof. In embodiments, aluminum, titanium, and zirconium may be used.

The ground plane 3 may be applied by known coating techniques, such as solution coating, vapor deposition, and sputtering. A method of applying an electrically conductive ground plane is by vacuum deposition. Other suitable methods may also be used.

### The Charge Blocking Layer

After deposition of any electrically conductive ground plane layer, a charge blocking layer 4 may be applied thereto. Electron blocking layers for positively charged photoreceptors permit holes from the imaging surface of the photoreceptor to migrate toward the conductive layer. For negatively charged photoreceptors, any suitable hole blocking layer capable of forming a barrier to prevent hole injection from the conductive layer to the opposite photoconductive layer may be utilized.

If a blocking layer is employed, it may be positioned over the electrically conductive layer. The term "over," as used herein in connection with many different types of layers, should be understood as not being limited to instances wherein the layers are contiguous. Rather, the term "over" refers, for example, to the relative placement of the layers and encompasses the inclusion of unspecified intermediate layers.

The blocking layer 4 may include polymers such as polyvinyl butyral, epoxy resins, polyesters, polysiloxanes, polyamides, polyurethanes, and the like; nitrogen-containing siloxanes or nitrogen-containing titanium compounds, such as trimethoxysilyl propyl ethylene diamine, N-beta(aminoethyl) gamma-aminopropyl trimethoxy silane, isopropyl 4-aminobenzene sulfonyl titanate, di(dodecylbenezene sulfonyl) titanate, isopropyl di(4-aminobenzoyl)isostearoyl titanate, isopropyl tri(N-ethyl amino) titanate, isopropyl trianthranil titanate, isopropyl tri(N,N-dimethyl-ethyl amino) titanate, titanium-4-amino benzene sulfonate oxyacetate, titanium 4-aminobenzoate isostearate oxyacetate, gamma-aminobutyl methyl dimethoxy silane, gamma-aminopropyl methyl dimethoxy silane, and gamma-aminopropyl trimethoxy silane, as disclosed in U.S. Pat. Nos. 4,338,387; 4,286,033; and 4,291,110 the disclosures of which are incorporated herein by reference in their entireties.

The phrase "n-type" refers, for example, to materials which predominately transport electrons. Typical n-type materials include dibromoanthanthrone, benzimidazole perylene, zinc oxide, titanium oxide, azo compounds such as chlorodiane blue and bisazo pigments, substituted 2,4-dibromotriazines, polynuclear aromatic quinones, zinc sulfide, and the like.

The phrase "p-type" refers, for example, to materials which transport holes. Typical p-type organic pigments include, for example, metal-free phthalocyanine, titanyl phthalocyanine, gallium phthalocyanine, hydroxy gallium phthalocyanine, chlorogallium phthalocyanine, copper phthalocyanine, and the like.

### The Adhesive Layer

An intermediate layer 5 between the blocking layer 4 and the charge generating 6 layer may, if desired, be provided to promote adhesion. However, in embodiments, a dip coated aluminum drum may be utilized without an adhesive layer.

Additionally, adhesive layers may be provided, if necessary, between any of the layers in the photoreceptors to ensure adhesion of any adjacent layers. Alternatively, or in addition, adhesive material may be incorporated into one or both of the respective layers to be adhered.

### The Imaging Layer(s)

The imaging layer refers to a layer or layers containing charge generating material, charge transport material, or both the charge generating material and the charge transport material.

Either a n-type or a p-type charge generating material may be employed in the present photoreceptor.

### Charge Generation Layer

Illustrative organic photoconductive charge generating materials include azo pigments such as Sudan Red, Dian Blue, Janus Green B, and the like; quinone pigments such as Algol Yellow, Pyrene Quinone, Indanthrene Brilliant Violet RRP, and the like; quinocyanine pigments; perylene pigments such as benzimidazole perylene; indigo pigments such as indigo, thioindigo, and the like; bisbenzoimidazole pigments such as Indofast Orange, and the like; phthalocyanine pigments such as copper phthalocyanine, aluminochloro-phthalocyanine, hydroxygallium phthalocyanine, chlorogallium phthalocyanine, titanyl phthalocyanine and the like; quinacridone pigments; or azulene compounds. Suitable inorganic photoconductive charge generating materials include for example cadium sulfide, cadmium sulfoselenide, cadmium selenide, crystalline and amorphous selenium, lead oxide and other chalcogenides. In embodiments, alloys of selenium may be used and include for instance selenium-arsenic, selenium-tellurium-arsenic, and selenium-tellurium.

Any suitable inactive resin binder material may be employed in the charge generating layer. Typical organic resinous binders include polycarbonates, acrylate polymers, methacrylate polymers, vinyl polymers, cellulose polymers, polyesters, polysiloxanes, polyamides, polyurethanes, epoxies, polyvinylacetals, and the like.

### Charge Transport Layer

Additional charge transport materials include for example a positive hole transporting material selected from compounds having in the main chain or the side chain a polycyclic aromatic ring such as anthracene, pyrene, phenanthrene, coronene, and the like, or a nitrogen-containing hetero ring such as indole, carbazole, oxazole, isoxazole, thiazole, imidazole, pyrazole, oxadiazole, pyrazoline, thiadiazole, triazole, and hydrazone compounds. Typical hole transport materials include electron donor materials, such as carbazole; N-ethyl carbazole; N-isopropyl carbazole; N-phenyl carbazole; tetraphenylpyrene; 1-methylpyrene; perylene; chrysene; anthracene; tetraphene; 2-phenyl naphthalene; azopyrene; 1-ethyl pyrene; acetyl pyrene; 2,3-benzochrysene; 2,4-benzopyrene; 1,4-bromopyrene; poly(N-vinylcarbazole); poly(vinylpyrene); poly(vinyltetraphene); poly(vinyltetracene) and poly(vinylperylene). Suitable electron transport materials include electron acceptors such as 2,4,7-trinitro-9-fluorenone; 2,4,5,7-tetranitro-fluorenone; dinitroanthracene; dinitroacridene; tetracyanopyrene; dinitroanthraquinone; and butylcarbonylfluorenemalononitrile, see U.S. Pat. No. 4,921,769 the disclosure of which is incorporated herein by reference in its entirety. Other hole transporting materials include arylamines described in U.S. Pat. No. 4,265,990 the disclosure of which is incorporated herein by reference in its entirety, such as N,N'-diphenyl-N,N'-bis(alkylphenyl)-(1,1'-biphenyl)-4,4'-diamine wherein alkyl is selected from the group consisting of methyl, ethyl, propyl, butyl, hexyl, and the like. Other known charge transport layer molecules may be selected, reference for example U.S. Pat. Nos. 4,921,773 and 4,464,450 the disclosures of which are incorporated herein by reference in their entireties.

### Overcoat Layer

Embodiments in accordance with the present disclosure can include an overcoat layer or layers 8, which are positioned over the charge generation layer or over the charge transport layer. This layer incudes FSOFs disclosed herein.

Such a protective overcoating layer includes a FSOF forming reaction mixture containing a plurality of molecular building blocks that optionally contain charge transport segments.

Additives may be present in the overcoating layer in the range of about 0.5 to about 40 weight percent of the overcoating layer. In embodiments, additives include organic and inorganic particles which can further improve the wear resistance and/or provide charge relaxation property. In embodiments, organic particles include Teflon powder, carbon black, and graphite particles. In embodiments, inorganic particles include insulating and semiconducting metal oxide particles such as silica, zinc oxide, tin oxide and the like. Another semiconducting additive is the oxidized oligomer salts as described in U.S. Pat. No. 5,853,906 the disclosure of which is incorporated herein by reference in its entirety. In embodiments, oligomer salts are oxidized N,N,N',N'-tetra-p-tolyl-4,4'-biphenyldiamine salt.

Overcoating layers from about 2 micrometers to about 15 micrometers, such as from about 3 micrometers to about 8 micrometers are effective in preventing charge transport molecule leaching, crystallization, and charge transport layer cracking in addition to providing scratch and wear resistance.

### The Ground Strip

The ground strip 9 may comprise a film-forming binder and electrically conductive particles. Cellulose may be used to disperse the conductive particles. Any suitable electrically conductive particles may be used in the electrically conductive ground strip layer 8. The ground strip 8 may, for example, comprise materials that include those enumerated in U.S. Pat. No. 4,664,995 the disclosure of which is incorporated herein by reference in its entirety. Typical electrically conductive particles include, for example, carbon black, graphite, copper, silver, gold, nickel, tantalum, chromium, zirconium, vanadium, niobium, indium tin oxide, and the like.

In embodiments, a SOF may be incorporated into various components of an image forming apparatus. For example, a SOF may be incorporated into a electrophotographic photoreceptor, a contact charging device, an exposure device, a developing device, a transfer device and/or a cleaning unit. In embodiments, such an image forming apparatus may be equipped with an image fixing device, and a medium to which an image is to be transferred is conveyed to the image fixing device through the transfer device.

The contact charging device may have a roller-shaped contact charging member. The contact charging member may be arranged so that it comes into contact with a surface of the photoreceptor, and a voltage is applied, thereby being able to give a specified potential to the surface of the photoreceptor. In embodiments, a contact charging member may be formed from a SOF and or a metal such as aluminum, iron or copper, a conductive polymer material such as a polyacetylene, a polypyrrole or a polythiophene, or a dispersion of fine particles of carbon black, copper iodide, silver iodide, zinc sulfide, silicon carbide, a metal oxide or the like in an elastomer material such as polyurethane rubber, silicone rubber, epichlorohydrin rubber, ethylenepropylene rubber, acrylic rubber, fluororubber, styrene-butadiene rubber or butadiene rubber.

In embodiments an optical device that can perform desired imagewise exposure to a surface of the electrophotographic photoreceptor with a light source such as a semiconductor laser, an LED (light emitting diode) or a liquid crystal shutter, may be used as the exposure device.

In embodiments, a known developing device using a normal or reversal developing agent of a one-component system, a two-component system or the like may be used in embodiments as the developing device. There is no particular limitation on image forming material (such as a toner, ink or the like, liquid or solid) that may be used in embodiments of the disclosure.

Contact type transfer charging devices using a belt, a roller, a film, a rubber blade or the like, or a scorotron transfer charger or a scorotron transfer charger utilizing corona discharge may be employed as the transfer device, in various embodiments. In embodiments, the charging unit may be a biased charge roll, such as the biased charge rolls.

Further, in embodiments, the cleaning device may be a device for removing a remaining image forming material, such as a toner or ink (liquid or solid), adhered to the surface of the electrophotographic photoreceptor after a transfer step, and the electrophotographic photoreceptor repeatedly subjected to the above-mentioned image formation process may be cleaned thereby. In embodiments, the cleaning device may be a cleaning blade, a cleaning brush, a cleaning roll or the like. Materials for the cleaning blade include SOFs or urethane rubber, neoprene rubber and silicone rubber.

In an exemplary image forming device, the respective steps of charging, exposure, development, transfer and cleaning are conducted in turn in the rotation step of the electrophotographic photoreceptor, thereby repeatedly performing image formation. The electrophotographic photoreceptor may be provided with specified layers comprising SOFs and photosensitive layers that comprise the desired SOF, and thus photoreceptors having excellent discharge gas resistance, mechanical strength, scratch resistance, particle dispersibility, etc., may be provided. Accordingly, even in embodiments in which the photoreceptor is used together with the contact charging device or the cleaning blade, or further with spherical toner obtained by chemical polymerization, good image quality may be obtained without the occurrence of image defects such as fogging. That is, embodiments of the invention provide image-forming apparatuses that can stably provide good image quality for a long period of time is realized.

Further, in embodiments, the cleaning device may be a device for removing a remaining image forming material, such as a toner or ink (liquid or solid), adhered to the surface of the electrophotographic photoreceptor after a transfer step, and the electrophotographic photoreceptor repeatedly subjected to the above-mentioned image formation process may be cleaned thereby. In embodiments, the cleaning device may be a cleaning blade, a cleaning brush, a cleaning roll or the like. Materials for the cleaning blade include SOFs or urethane rubber, neoprene rubber and silicone rubber.

While embodiments have been illustrated with respect to one or more implementations, alterations and/or modifications can be made to the illustrated examples without departing from the spirit and scope of the appended claims. In addition, while a particular feature herein may have been disclosed with respect to only one of several implementations, such feature may be combined with one or more other features of the other implementations as may be desired and advantageous for any given or particular function.

### EXAMPLES

### Comparative Example 1

A 40 mm commercially available production Xerox C75 drum photoreceptor without a protective FSOF overcoat.

### Comparative Example 2

A 30 mm commercially available Hodaka F469 drum photoreceptor without a protective FSOF overcoat.

### Comparative Example 3

### Preparation of Liquid Containing Reaction mixture

The following were combined: a first building block N4,N4,N4',N4'-tetrakis(4-(methoxymethyl)phenyl)biphenyl-4,4'-diamine, a second building block 1H,1H,8H,8H-Dodecafluoro-1,8-octanediol, an acid catalyst 20 wt % solution ofNacure XP-357, a leveling agent 25 wt % solution of Silclean 3700, an optional anti-oxidant TrisTPM, and a solvent 1-methoxy-2-propanol. The resulting solution was mixed and filtered using a 1 micron PTFE filter.

### Deposition of Reaction Mixture

The solution was coated onto a commercially available production Xerox C75 drum photoreceptor (40mm drum) and a commercially available Hodaka F469 drum photoreceptor (30mm drum) and then dried in a forced air oven at about 135°C for about 40 minutes. The resulting cured FSOF overcoat layer was about 4 microns thick and wherein the fluorinated segment 1H,1H,8H,8H-Dodecafluoro-1,8-octanediol is greater than 25 weight percent of the FSOF layer.

### Example 1

The following were combined: a first building block N4,N4,N4',N4'-tetrakis(4-(methoxymethyl)phenyl)biphenyl-4,4'-diamine, a second building block 1H,1H,8H,8H-Dodecafluoro-1,8-octanediol, an acid catalyst 20 wt % solution ofNacure XP-357, a leveling agent 25 wt % solution of Silclean 3700, an optional anti-oxidant TrisTPM, and a solvent 1-methoxy-2-propanol. The resulting solution was mixed and filtered using a 1 micron PTFE filter.

### Deposition of Reaction Mixture

The solution was coated onto a Xerox C75 drum photoreceptor (40mm drum) and a Hodaka F469 drum photoreceptor (30mm drum) and then dried in a forced air oven at about 155°C for about 40 minutes. The resulting cured FSOF overcoat layer was about 4 microns thick and wherein the fluorinated segment 1H,1H,8H,8H-Dodecafluoro-1,8-octanediol is about 10 weight percent of the FSOF layer.

### Example 2

The following were combined: a first building block N4,N4,N4',N4'-tetrakis(4-(methoxymethyl)phenyl)biphenyl-4,4'-diamine, a second building block 1H,1H,8H,8H-Dodecafluoro-1,8-octanediol, an acid catalyst 20 wt % solution ofNacure XP-357, a leveling agent 25 wt % solution of Silclean 3700, an optional anti-oxidant TrisTPM, and a solvent 1-methoxy-2-propanol. The resulting solution was mixed and filtered using a 1 micron PTFE filter.

### Deposition of Reaction Mixture

The solution was coated onto a Xerox C75 drum photoreceptor (40mm drum) and a Hodaka F469 drum photoreceptor (30mm drum) and then dried in a forced air oven at about 165°C for about 40 minutes. The resulting cured FSOF overcoat layer was about 4 microns thick and wherein the fluorinated segment 1H,1H,8H,8H-Dodecafluoro-1,8-octanediol is about 5 weight percent of the FSOF layer.

### Evaluations, Results and Discussion

Wear rate was measured for each 30mm drum in a wear test fixture for 50kcyc. Comparative example 2 (no overcoat) wear rate was measured to be ∼92nm/kcyc. Comparative Example 3 (high fluorine content) wear rate was ∼21.8nm/kcyc. Example 1 wear rate was ∼15.6nm/kcyc. Example 2 wear rate was ∼ 8.6nm/kcyc. There was a dramatic reduction in wear rate as the fluorine segment content is reduced.

40mm drums were print tested continuously in a Xerox Color J75 printer for 120,000 prints and FSOF thickness loss was measured and wear rate calculated. Comparative Example 1 (no overcoat) wear rate was ∼25.6nm/kcyc. Example 2 (5 weight percent fluorine building block) wear rate was ∼1nm/kcyc. The in-machine wear rate of Example 2 is low enough to enable several million cycles before the overcoat is completely worn away.

40mm drums were tested for image quality (IQ) in a Xerox J75 Printer for up to 120,000 prints. All examples demonstrated no LCM, ghosting or background issues and delivered good image quality even after 120,000 prints.

By reducing the fluorine segment content the wear rate can be dramatically increased. This enables a typical 4-5 micron overcoat layer to last several million prints before being worn away. Furthermore, reducing the fluorine content to low levels does not introduce issues like torque, LCM, or background.

It will be appreciated that variants of the above-disclosed and other features and functions or alternatives thereof may be combined into other different systems or applications. Various presently unforeseen or unanticipated alternatives, modifications, variations, or improvements therein may be subsequently made by those skilled in the art, which are also encompassed by the following claims.

## Claims

1. An imaging member comprising:
a substrate;
a charge generating layer;
a charge transport layer; and
an outermost layer comprising a structured organic film (SOF) comprising a fluorinated molecular building block and a hole molecular building block, wherein the fluorinated molecular building block is present in the SOF of the outermost layer in an amount of from about 1 weight percent to about 20 weight percent of the SOF.

2. The imaging member of claim 1, wherein the fluorinated molecular building block and the hole molecular building block are present in the SOF of the outermost layer in an amount of from about 90 to about 99.5 percent by weight of the SOF.

3. The imaging member of claim 1, wherein the outermost layer is an overcoat layer, and the overcoat layer is from about 2 to about 10 microns thick.

4. The imaging member of claim 1, wherein the fluorinated molecular building block is selected from the group consisting of: α, ω-fluoroalkyldiols of the general structure: where n is an integer having a value of from 1 to about 100; fluorinated alcohols of the general structure HOCH₂(CF₂)ₙCH₂OH where n is an integer having a value of from 1 to about 100; tetrafluorohydroquinone; perfluoroadipic acid hydrate, 4,4'-(hexafluoroisopropylidene)diphthalic anhydride; and 4,4'-(hexafluoroisopropylidene)diphenol.

5. The imaging member of claim 1, wherein the fluorinated molecular building block is selected from the group consisting of: 1,1,8,8-dodecafluoro-1,8-octanediol, 2,2,3,3,4,4,5,5-octafluoro-1,6-hexanediol, 2,2,3,3,4,4,5,5,6,6,7,7-dodecanfluoro-1,8-octanediol, 2,2,3,3,4,4,5,5,6,6,7,7,8,8,9,9-perfluorodecane-1,10-diol, (2,3,5,6-tetrafluoro-4-hydroxymethyl-phenyl)-methanol, 2,2,3,3-tetrafluoro-1,4-butanediol, 2,2,3,3,4,4-hexafluoro-1,5-pentanedial, and 2,2,3,3,4,4,5,5,6,6,7,7,8,8-tetradecafluoro-1,9-nonanediol.

6. An electrostatographic apparatus comprising:
an imaging member, having an outermost layer that comprises a structured organic film (SOF) comprising a plurality of fluorinated molecular building blocks and a plurality of hole molecular building blocks, wherein the fluorinated molecular building blocks are present in the SOF in an amount of from about 1 weight percent to about 20 weight percent of the SOF;
a charging unit to impart an electrostatic charge on the imaging member; an exposure unit to create an electrostatic latent image on the imaging member;
an image material delivery unit to create an image on the imaging member; a transfer unit to transfer the image from the imaging member; and
an optional cleaning unit.

7. The electrostatographic apparatus of claim 6, wherein the charging unit is a biased charge roll.

8. An imaging member comprising:
a substrate;
a charge generating layer;
a charge transport layer; and
an outermost layer comprising a structured organic film (SOF) comprising fluorinated molecular building blocks and hole molecular building blocks, wherein the fluorinated molecular building blocks are present in the SOF in an amount of from about 1 weight percent to about 10 weight percent of the SOF.

9. The imaging member of claim 8, wherein the fluorinated molecular building block is selected from the group consisting of: 1,1,8,8-dodecafluoro-1,8-octanediol, 2,2,3,3,4,4,5,5-octafluoro-1,6-hexanediol, 2,2,3,3,4,4,5,5,6,6,7,7-dodecanfluoro-1,8-octanediol, 2,2,3,3,4,4,5,5,6,6,7,7,8,8,9,9-perfluorodecane-1,10-diol, (2,3,5,6-tetrafluoro-4-hydroxymethyl-phenyl)-methanol, 2,2,3,3-tetrafluoro-1,4-butanediol, 2,2,3,3,4,4-hexafluoro-1,5-pentanedial, and 2,2,3,3,4,4,5,5,6,6,7,7,8,8-tetradecafluoro-1,9-nonanediol.

10. The imaging member of claim 8, wherein the hole transport building block is selected from the group consisting of N4,N4,N4',N4'-tetrakis(4-(methoxymethyl)phenyl)biphenyl-4,4'-diamine N,N,N',N'-tetra-(p-tolyl)biphenyl-4,4'-diamine: and N4,N4'-bis(3,4-dimethylphenyl)-N4,N4'-dip-tolyl-[1,1'-biphenyl]-4,4'-diamine.
